

## UNITED STATES PATENT OFFICE

2,451,426

## BRIGHT ZINC PLATING

Robert R. Bair and Harry L. Benner, Niagara Falls, and Joseph Frederic Walker, Lewiston, N. Y., assignors to E. I. du Pont de Nemours & Company, Wilmington, Del., a corporation of Delaware

No Drawing. Application November 25, 1943,  
Serial No. 511,686

4 Claims. (Cl. 204—55)

1

This invention relates to zinc plating and, more particularly, to the production of bright zinc electrodeposits.

A number of processes have been developed for plating bright zinc from cyanide baths by means of which excellent bright deposits can be obtained, provided the proper conditions such as temperature and current density are observed. An example of a successful bright zinc plating process is that described and claimed in U. S. Patent 2,171,842 wherein the bright deposit is obtained by the addition of a small amount of polyvinyl alcohol to the plating bath. This process produces very bright deposits of zinc and over a wide current density range at low temperatures such as 25 to 30° C. However, it is often desired to operate such a bath at higher temperatures, such as 50 to 60° C., whereby more rapid electroplating may be obtained. At such high temperatures the polyvinyl alcohol still functions as an excellent brightening agent, but the current density bright range at such high temperatures is materially limited. It is desirable, therefore, to have a brightening agent which will produce the bright deposits obtainable by means of polyvinyl alcohol and which can be employed for that purpose at elevated temperatures and over a wide current density range at such elevated temperatures.

Addition agents are often used heretofore in various acid zinc plating baths such as sulfate baths and chloride baths. The effect of such additions is to whiten the electrodeposit, but heretofore it has not been possible to produce lustrous, bright zinc plate from acid baths.

An object of the present invention is to provide an improved process for electroplating bright zinc deposits. A further object is to provide an addition agent for bright zinc plating baths which is operable over a wide range of temperatures and current density, and which is effective in alkaline, acidic and neutral zinc plating solutions. A further object is to provide an electroplating bath addition agent composition as hereinafter set forth. Still other objects will be apparent from the following description of our invention.

We have discovered that a certain polymeric condensation product of sodium cyanamide and formaldehyde, which is soluble in alkaline solutions having a pH above 9 and insoluble in water at a pH of 8 to 9, is an excellent brightening agent for zinc plating baths, whether alkaline, acidic or neutral. We have further discovered that when this condensation product is added to an alkaline zinc plating bath which already contains

2

a polyvinyl alcohol addition agent, excellent bright deposits can be obtained over a wide range of current densities at temperatures from 20° C. to as high as 60° C. and even higher. In other words, the addition of the condensation product widens the current density bright range at the higher temperatures.

The aforesaid condensation product is described and claimed in a copending patent application, Serial No. 507,182, filed October 21, 1943 by Joseph F. Walker, now Patent No. 2,411,396. This condensation product may be made by the addition of sodium cyanamide to aqueous formaldehyde solutions, the reaction being carried out under alkaline conditions at a temperature below 35° C., preferably in the range of 15 to 20° C. The reaction between the cyanamide and the formaldehyde solution is exothermic and cooling is generally necessary to maintain the temperature below 35° C. After the reaction has been completed, the condensation product is precipitated from the reaction mixture by adding sufficient acid to reduce the alkalinity of the solution to a pH within the range 8 to 9. It may then be filtered off and dried, the pure product being a white powder.

The product is probably a partially hydrated polymer of methylene cyanamide ( $\text{CH}_2=\text{NCN}$ ) in which approximately two-thirds of the CN radicals have been converted to amide groups. Analyses for carbon, hydrogen, and nitrogen indicate that its composition closely approximates the empirical formula,  $\text{C}_6\text{H}_{10}\text{N}_2\text{O}_2$ . The characteristics of the product are those of an amorphous resin, and it is probably not a simple compound of low molecular weight but rather a polymer or mixture of polymers made up of units corresponding to the  $\text{C}_6\text{H}_{10}\text{N}_2\text{O}_2$  formula. It is believed that the structural formula of this polymer unit is as follows:



The new condensation product is a white, apparently non-crystalline solid which chars when heated to temperatures above 300° C. Although it is apparently stable when heated below 300° C. when dry, it undergoes further resinification when heated in the moist state and should be dried quickly and at relatively low temperatures to avoid undesirable alteration. On long heating in the moist state it combines with additional water and tends to liberate ammonia. A sample heated in this way was found to have an em-

pirical composition corresponding to  $C_8H_{12}N_6O_3$ .

The new product dissolves readily in dilute aqueous acids or strong alkalies and is relatively insoluble in pure water, the product being least soluble in aqueous liquids having a pH of 8.0-9.0. When dissolved in aqueous alkalies or acids it may be precipitated therefrom, although the yields upon reprecipitation are not entirely quantitative. Analyses of the reprecipitated product indicate that its composition is substantially unchanged.

In using this condensation product as a brightening agent, the amount to be added to the bath will vary upon the degree of brightening desired to be obtained. Generally, it is necessary to use at least about 0.1 ounce per gallon in order to obtain appreciable brightening effect. In amounts up to 2 ounces per gallon of the condensation product, excellent brightening is obtained over a wide range of current densities. Within this range generally the best results are obtained with a concentration of about 0.5 ounce per gallon. At concentrations above 2 ounces per gallon the brightening effect tends to occur only at relatively high cathode current density such as 50 to 500 amps. per sq. ft. Thus, when recessed articles are electroplated with such high concentration of the brightening agent, the areas of the cathode closest to the anode will plate bright, whereas the recesses which have a low current density tend to plate dull. With this limitation, our new brightening agent may be used in any concentration up to the limit of its solubility, which is approximately 16 ounces per gallon. If more of the addition agent is added than can dissolve in the plating bath, it is desirable to filter the bath to remove excess undissolved material, the presence of which will tend to cause roughness in the cathode deposit.

In practicing our invention by the conjoint addition of polyvinyl alcohol and the condensation product to an alkaline zinc plating bath, the amounts of polyvinyl alcohol suitable for zinc plating baths may be used, for example, the amounts shown in U. S. Patent 2,171,842. The optimum amount of polyvinyl alcohol will vary, and in most cases will lie in the range of 0.001 to 0.1 ounce per gallon. Generally we prefer to add not more than about 0.03 ounce per gallon of polyvinyl alcohol, e. g., 0.001 to 0.03 ounce per gallon in plating baths like those shown in the examples given hereinafter.

In a preferred method for practicing our invention, we prepare a mixture of polyvinyl alcohol and the condensation product containing 1 to 5% by weight of the polyvinyl alcohol, both substances being in the form of dry powders. A conventional zinc cyanide plating bath is then prepared by dissolving in water, zinc cyanide, sodium cyanide and caustic soda and this solution is purified so as to remove heavy metal ions, for example, by treatment with sodium sulfide or metallic zinc powder, followed by filtration if necessary. About  $\frac{1}{2}$  ounce per gallon of the above-described mixture of polyvinyl alcohol and condensation product is then dissolved in the plating bath. If desired, the dry addition agent may first be dissolved in water containing sufficient caustic soda to give a pH of 10 to 12. The resulting electroplating bath may then be operated in the conventional manner at any desired temperature, e. g. 25 to 60° C. and at cathode current densities up to 300 amps. per sq. ft.

The following examples further illustrate our invention:

#### Example 1

A zinc plating bath was made by dissolving the following ingredients in water:

|                     | Ounces per gallon |
|---------------------|-------------------|
| 5 Zinc cyanide..... | 8.0               |
| Sodium cyanide..... | 5.59              |
| Caustic soda.....   | 10.0              |

The solution was purified by the addition of  $\frac{1}{15}$  ounce per gallon of sodium sulfide. The bath was then operated to 40 amps. per sq. ft. at a temperature of 25° C. with pure zinc anodes. The resulting electrodeposit, after bright dipping in dilute nitric acid, was white but not bright. 20 grams per gallon of the condensation product of sodium cyanamide and formaldehyde was then added to the solution and when this had dissolved, the solution was again operated at 40 amps. per sq. ft. at 25° C. The electrodeposit after bright dipping had excellent brightness.

#### Example 2

A purified zinc plating solution was prepared as in Example 1 and to this was added 0.3 gram per gallon of polyvinyl alcohol in aqueous solution and 2.25 grams per gallon of the above-described condensation product. To determine the bright current density range of this plating bath, it was electrolyzed in a so-called Hull cell as described in Hull, U. S. Patent 2,149,344. These results showed that at the lower cathode current densities up to 6.5 amps. per sq. ft., the electrodeposit had a hazy white color. At current densities from 6.5 to 100 amps. per sq. ft. excellent bright plate was obtained. The bath was operated at a temperature of 30° C.

#### Example 3

To a zinc plating solution prepared as in Example 1, 4 grams per gallon of polyvinyl alcohol and 15 grams per gallon of the condensation product was added. With a bath temperature of 50° C. cathodic deposits were obtained at current densities from 20 to 180 amps. per sq. ft. which had excellent brightness after bright dipping in dilute nitric acid.

#### Example 4

The following zinc cyanide plating solution was made up:

|                     | Ounces per gallon |
|---------------------|-------------------|
| Zinc cyanide.....   | 8.0               |
| Sodium cyanide..... | 3.4               |
| Caustic soda.....   | 10.0              |

This was purified by addition of  $\frac{1}{15}$  ounce per gallon of sodium sulfide and  $\frac{1}{3}$  ounce per gallon of a mixture of the condensation product and powdered polyvinyl alcohol, containing 3% by weight of polyvinyl alcohol, was dissolved in the bath. This bath then was utilized to electroplate strip steel at cathode current densities of 200 to 300 amps. per sq. ft. After bright dipping, the resulting electrodeposits were bright and pleasing in appearance. The cathode current efficiencies were 90.5% at 200 amps. per sq. ft. and 69.5% at 300 amps. per sq. ft.

#### Example 5

To the zinc plating solution of Example 1 was added 9 grams per gallon of a mixture of equal parts by weight of the aforesaid condensation product and anisaldehyde. Excellent bright deposits were obtained at current densities of 3 to 120 amps. per sq. ft. With this bath good bright

deposits could be obtained without bright dipping.

*Example 6*

The method of Example 5 was repeated except that the zinc plating solution had the following formula:

|                | Ounces per gallon |
|----------------|-------------------|
| Zinc cyanide   | 8.0               |
| Sodium cyanide | 4.49              |
| Caustic soda   | 10.0              |

To this solution was added 0.5 ounce per gallon of the mixed addition agent described in Example 5. At current densities of 18 to 180 amps. per sq. ft. deposits were obtained which were bright and had a very slight bronze film. On bright dipping in dilute nitric acid, the bronze film was removed to produce an excellent bright surface.

*Example 7*

The following acidic zinc plating solution was prepared:

|                   |                   |      |
|-------------------|-------------------|------|
| Zinc chloride     | ounces per gallon | 18.0 |
| Ammonium chloride | do                | 28.0 |
| AlCl <sub>3</sub> | do                | 3.0  |
| pH adjusted to    | electrometric     | 3.5  |

The above solution, operated at 25° C., plated a white, crystalline, non-lustrous zinc deposit at current densities up to 150 amps. per sq. ft. An addition of 0.5 ounce per gallon of the herein-described condensation product gave an excellent bright zinc deposit at current densities of about 40 to 125 amps. per sq. ft.

*Example 8*

A sodium zincate bath was prepared as follows:

|                | Ounces per gallon |
|----------------|-------------------|
| Zinc hydroxide | 7.5               |
| Caustic soda   | 20.0              |

This solution, operated at 30° C., produced a white, crystalline, non-lustrous zinc plate at current densities of 4 to 10 amps. per sq. ft. At higher current densities, the deposits were gray and spongy. An addition of 1 ounce per gallon of a mixture of 97 parts by weight of the condensation product and 3 parts by weight of polyvinyl alcohol gave a semi-bright, lustrous deposit at current densities of 10 to 100 amps. per sq. ft.

*Example 9*

A zinc sulfate bath was prepared as follows:

|                   |                   |      |
|-------------------|-------------------|------|
| Zinc sulfate      | ounces per gallon | 32.0 |
| Ammonium chloride | do                | 2.0  |
| Aluminum sulfate  | do                | 4.0  |
| pH adjusted to    | electrometric     | 3.25 |

Without addition agent deposits plated from this solution at a bath temperature of 25° C. were gray to white matte and at current densities in excess of approximately 125 amps. per sq. ft., the deposits were dark gray. The addition of 0.5 ounce per gallon of the condensation product gave brilliant, lustrous deposits at current densities of 10 to above 125 amps. per sq. ft.

*Example 10*

A zinc pyrophosphate plating bath was prepared as follows:

|                               |                   |      |
|-------------------------------|-------------------|------|
| Zinc pyrophosphate            | ounces per gallon | 8.0  |
| Sodium sulfate                | do                | 4.0  |
| NH <sub>4</sub> OH to a pH of | electrometric     | 11.5 |

This bath was operated at a bath temperature of

30° C. The deposits were dark gray at current densities of 10 to 25 amps. per sq. ft. and spongy and non-adherent at higher current densities. The addition of 1 ounce per gallon of the mixed addition agent of Example 8 gave pleasing white, lustrous zinc deposits at current densities of 10 to 60 amps. per sq. ft.

Our invention also includes the novel zinc plating addition agent which comprises a mixture of the condensation product and polyvinyl alcohol in suitable proportions. The preferred composition is made by mixing the solid, pulverulent condensation product with anhydrous, finely divided polyvinyl alcohol so that the mixture contains 1 to 5% by weight of the polyvinyl alcohol. This may be dissolved in caustic soda solution or other aqueous alkaline liquid to prepare a stock solution. We have found the two ingredients to be mutually compatible, and substantially non-reactive towards each other, both in the anhydrous state and in solution. If desired, other substances may be added to the mixture, either in solid or in solution form, for example, plating bath ingredients, other addition agents, dyes or pigments, or inert materials. Excellent results have been obtained with a pulverulent mixture containing approximately 3% by weight of polyvinyl alcohol and 97% by weight of the condensation product.

As shown by the foregoing examples, our novel brightening agent may be used in zinc plating baths either alone or in combination with other brightening agents, including both organic agents and metallic compounds such as salts of molybdenum, manganese, chromium and the like. As the condensation product has a low solubility at a pH of 8 to 9, it is preferable that the plating bath have a pH below 8 or higher than 9. This presents no difficulty as alkaline zinc cyanide plating baths usually have the required high pH and the acid to neutral baths have a pH below 8. While we prefer to utilize our addition agent in zinc cyanide baths, which have been purified to remove heavy metal ions, the invention is not restricted thereto as improved electrodeposits are obtained in baths which have not been so purified.

Likewise, the invention is not restricted to the bath formulas shown in the above examples, which have been given merely by way of example. Our novel brightening agent is effective for electroplating from any aqueous solution containing a zinc compound in solution. In baths which inherently produce inferior zinc deposits, the appearance of the deposit is invariably improved by addition of our condensation product. Baths which inherently produce superior zinc deposits generally are markedly improved by means of our addition agent and are preferred in practicing our invention. Thus, to produce bright, lustrous zinc deposits according to our invention, we generally prefer to utilize the zinc chloride and zinc sulfate acid baths and the zinc cyanide alkaline baths.

Suitable zinc cyanide baths may be made, for example, by dissolving zinc cyanide, oxide or carbonate in a solution of an alkali metal cyanide. While we prefer to use sodium or potassium cyanide, the cyanides of other alkali metals, cesium, rubidium and lithium may be used if desired. The bath may contain the ions of one or several of the alkali metals in any desired proportions. The presence of caustic soda or other alkali metal hydroxide, while generally desirable, is not essential in practicing our invention.

In common with most alkaline bright zinc plat-

ing processes, the electrodeposit obtained from a cyanide bath by our process may have more or less of a brownish or bronze-like film which can readily be removed by conventional bright dipping procedures to obtain maximum brightness. In some cases the film is so slight that bright dipping is not necessary or desirable, and our invention is not restricted to the use of a bright dip operation. If bright dipping is desired, any of the conventional zinc bright dips can be used, for example, dilute nitric acid, acidified peroxide solutions or other oxidizing acid solutions.

In electroplating zinc from acidic zinc chloride or zinc sulfate solutions, we prefer to have present in the bath a small amount of an aluminum salt, for example, 1 to 10 ounces per gallon of aluminum chloride or aluminum sulfate.

While we prefer to use the herein-described invention to electrodeposit pure zinc, the invention is not restricted thereto. If desired, various metal salts may be included in the plating bath to brighten or otherwise modify the cathodic deposit and the electrodeposit then may contain up to 10% by weight of such added metal. Thus, the invention may be used to produce improved electrodeposits composed of 90% or more by weight of zinc. Representative examples of such other metallic components which may be thus codeposited are molybdenum, chromium, manganese, copper, silver, mercury and cadmium. 30

We claim:

1. The process of electrodepositing zinc from an aqueous zinc cyanide electroplating solution having a pH above 9.0 which comprises electrodepositing said zinc from said solution containing dissolved therein about 0.1 to 2.0 ounces per gallon of the condensation product of sodium cyanamide and formaldehyde obtained by reacting substantially equimolecular amounts of sodium cyanamide and formaldehyde in aqueous alkaline solution at a temperature below 35° C. 35

2. The process of electrodepositing zinc from an aqueous zinc cyanide electroplating solution having a pH above 9.0 which comprises electrodepositing said zinc from said solution containing dissolved therein about 0.1 to 2.0 ounces per 45 gallon of the condensation product of sodium cyanamide and formaldehyde obtained by react-

ing substantially equimolecular amounts of sodium cyanamide and formaldehyde in aqueous alkaline solution at a temperature below 35° C., and about 0.001 to 0.1 ounce per gallon of polyvinyl alcohol.

3. An aqueous zinc electroplating solution containing the necessary components for the electrodeposition of zinc, said solution having a pH above 9.0 and containing dissolved therein as a brightening agent, 0.1 to 2.0 ounces per gallon of the condensation product of sodium cyanamide and formaldehyde obtained by reacting substantially equimolecular amounts of sodium cyanamide and formaldehyde in aqueous alkaline solution at a temperature below 35° C.

4. An aqueous zinc electroplating solution containing the necessary components for the electrodeposition of zinc, said solution having a pH above 9.0 and containing dissolved therein as a brightening agent, 0.1 to 2.0 ounces per gallon of the condensation product of sodium cyanamide and formaldehyde obtained by reacting substantially equimolecular amounts of sodium cyanamide and formaldehyde in aqueous alkaline solution at a temperature below 35° C., and 0.001 to 0.1 ounce per gallon of polyvinyl alcohol.

ROBERT R. BAIR.

HARRY L. BENNER.

JOSEPH FREDERIC WALKER.

#### REFERENCES CITED

The following references are of record in the file of this patent:

#### UNITED STATES PATENTS

| Number    | Name           | Date          |
|-----------|----------------|---------------|
| 1,791,434 | Schmidt        | Feb. 3, 1931  |
| 2,101,580 | Hendricks      | Dec. 7, 1937  |
| 2,111,698 | Seifert        | Feb. 22, 1938 |
| 2,171,842 | Barrett et al. | Sept. 5, 1939 |
| 2,288,318 | Hoffman        | June 30, 1942 |
| 2,328,593 | Widmer         | Sept. 7, 1943 |
| 2,411,396 | Walker         | Nov. 19, 1946 |
| 2,411,397 | Walker         | Nov. 19, 1946 |

#### OTHER REFERENCES

Metal Industry, Nov. 29, 1940, page 443.